

## UNITED STATES PATENT OFFICE

CAMILLE DREYFUS, OF NEW YORK, N. Y., AND HERBERT PLATT, OF CUMBERLAND, MARYLAND, ASSIGNEES TO CELANESE CORPORATION OF AMERICA, A CORPORATION OF DELAWARE

## CELLULOSE FIBERS, FABRICS AND ARTICLES

No Drawing.

Application filed September 22, 1925. Serial No. 57,956.

We have found the surprising fact that in treating cellulose derivatives, like cellulose acetate or other ethers or esters of cellulose, with stannic chloride under certain conditions and precipitating an insoluble tin salt in the fiber, a substantial increase in weight and volume of the fiber takes place without impairing or substantially impairing the aspect or other qualities of the fibers, fabrics or articles containing this fiber. The invention can best be illustrated by the following examples:

*Example No. 1.*—One (1) part of artificial silk made from cellulose acetate is treated with thirty (30) parts of 40° Tw. solution of stannic chloride ( $SnCl_4$ ) during one-half ( $\frac{1}{2}$ ) hour, at a temperature between 40° and 50° C., then rinsed off in water, then treated with 7° Tw. solution of di-sodium hydrogen phosphate ( $Na_2HPO_4$ ), and rinsed again, and then treated with 7° Tw. solution of sodium silicate, and washed with or without soap solution. The result will be a substantial increase in weight and volume of the fibers, fabrics and articles.

*Example No. 2.*—One (1) part of cellulose acetate artificial silk is treated with thirty (30) parts of stannic chloride solution of 40° Tw., at a temperature between 45° and 55° C., during one-half ( $\frac{1}{2}$ ) hour. Then rinse off in water and treat with sodium silicate 7° Tw. and wash with or without soap solution. The result will be a substantial increase in weight and volume of the fibers, fabrics and articles.

*Example No. 3.*—One (1) part of cellulose acetate artificial silk is treated with thirty (30) parts of 40° Tw. solution of stannic chloride, during one-half ( $\frac{1}{2}$ ) hour, at a temperature between 55° and 65° C., then rinsed off in water and treated with 7° Tw. sodium silicate solution, and washed with or without soap solution. The increase in weight and volume is larger in this case than under Example No. 2.

These examples are only descriptive and not limited and the temperature, as well as the time, can be varied within limits, as well as the strength of the stannic chloride and di-sodium hydrogen phosphate and sodium silicate solution within limits. In case, for instance, the temperature should be raised, it is advantageous to reduce the time of action of the stannic chloride. Instead of stannic chloride other metal salts, like zinc chloride, can be used, which are swelling agents for the cellulose acetate or for the cellulose ester or cellulose ethers, or other metal salts can also be used which are only slight swelling agents for the particular fiber, when they are used in conjunction with a swelling agent of the particular fiber. This process can be applied to the fiber itself as well as to a fabric made out of this fiber; for instance a fabric made of 100% cellulose acetate silk. The operations described in above examples can be repeated once or several times if it is desired to get a larger increase of volume and weight.

This process has a very beneficial effect on cellulose acetate fabrics. Apart from the increase of volume and weight it reduces the slipping of the fabrics and it conveys to the fabrics a fire-proof character or rather very heat resistant character, as it is a well known fact that cellulose acetate silk fabrics melt with a too hot an iron. After the application of this treatment no such melting takes place by treatment with a hot iron. It also reduces the inflammability of the fibers, fabrics and articles. Furthermore, for instance, a circular knitted fabric made with cellulose acetate silk and treated according to this process will show reduction in the laddering capacity of the fabric when treated according to the above process.

Instead of cellulose acetate, other cellulose esters of organic nature, or cellulose ethers can be used such as the butyrate, propionate, methylate, or ethylate of cellulose, and this process can be done with the fiber alone or

fabrics consisting of 100% cellulose acetate or cellulose esters or ethers, or fabrics containing partly cellulose acetate and partly other fibers like silk, etc.

5 For convenience the fibers, fabrics or other articles will be designated in the claims as materials. Also to avoid alternativeness of expression, the cellulose esters, ethers, and the like, will be generically termed organic substitution derivatives of cellulose.

10 Instead or partly instead of di-sodium hydrogen phosphate and sodium silicate, tannic acid can be used in above examples.

15 The term "weighting" is used in the appended claims in the ordinary technical signification in which it is employed in connection with natural silk, that is to say, to denote the operation of increasing the weight and volume of the material under treatment; 20 it does not include the production of such relatively small increases in weight as may be associated with processes of dyeing, such for example as those effected with the aid of mordants.

25 What we claim is:

1. A process for the weighting of material comprising an organic derivative of cellulose, which consists in swelling and impregnating said material with a salt of a weighting metal in solution, and subsequently treating to fix the metal in said material as an insoluble salt.

2. A process for the weighting of material comprising an organic derivative of cellulose, which consists in swelling and impregnating said material with a salt of a weighting metal in solution, and subsequently fixing the metal in said material as an insoluble silicate.

3. A process for the weighting of material comprising an organic derivative of cellulose, which consists in swelling and impregnating said material with a salt of a weighting metal in solution, and subsequently treating with a soluble phosphate and a soluble silicate to fix the metal in said material in the form of its corresponding insoluble salts.

4. A process for the weighting of material comprising an organic derivative of cellulose, which consists in swelling and impregnating said material with a chloride of a weighting metal in solution, and subsequently treating to fix the metal in said material as an insoluble salt.

5. A process for the weighting of material comprising an organic derivative of cellulose, which consists in swelling and impregnating said material with a chloride of a weighting metal in solution, and subsequently treating with alkali silicate to fix the metal in said material as an insoluble silicate.

6. A process for the weighting of material comprising an organic derivative of cellulose, which consists in swelling and impregnating said material with a chloride of a weighting metal in solution, and subsequently treating

with an alkali phosphate and an alkali silicate to fix the metal in said material in the form of its corresponding insoluble salts.

7. A process for the weighting of material comprising an organic derivative of cellulose, which consists in swelling and impregnating said material at a temperature of from 40-65° C. with a chloride of a weighting metal in solution, and subsequently fixing the metal in said material as an insoluble salt. 75

8. A process for the weighting of material comprising an organic derivative of cellulose, which consists in swelling and impregnating said material with stannic chloride in solution, and subsequently treating to fix the tin in said material as an insoluble salt. 80

9. A process for the weighting of material comprising an organic derivative of cellulose, which consists in swelling and impregnating said material with stannic chloride in solution, and subsequently treating with alkali silicate to fix the tin in said material as an insoluble silicate. 85

10. A process for the weighting of material comprising an organic derivative of cellulose, which consists in swelling and impregnating said material with stannic chloride in solution, and subsequently treating with an alkali phosphate and an alkali silicate to fix the tin in said material in the form of its corresponding insoluble salts. 90

11. A process for the weighting of material comprising an organic derivative of cellulose, which consists in swelling and impregnating said material at a temperature of from 40-65° C. with stannic chloride in solution, and subsequently fixing the tin in said material as an insoluble salt. 100

12. A process for the weighting of material comprising an organic derivative of cellulose, which consists in swelling and impregnating said material at a temperature of from 40-65° C. with stannic chloride in solution, and subsequently fixing the tin in said material as an insoluble silicate. 105

13. A process for the weighting of material comprising an organic derivative of cellulose, which consists in swelling and impregnating said material at a temperature of from 40-65° C. with stannic chloride in solution, and subsequently treating with a soluble phosphate and a soluble silicate to fix the tin in said material in the form of its corresponding insoluble salts. 115

14. A process for the weighting of material comprising an organic derivative of cellulose, which consists in swelling and impregnating said material at a temperature of from 40-65° C. with stannic chloride in solution, and subsequently treating at a lower temperature to fix the tin in said material as an insoluble salt. 120

15. A process for the weighting of material comprising cellulose acetate, which consists in swelling and impregnating said ma- 130

- terial with a salt of a weighting metal in solution, and subsequently treating to fix the metal in said material as an insoluble salt.
16. A process for the weighting of material comprising cellulose acetate, which consists in swelling and impregnating said material with a salt of a weighting metal in solution, and subsequently fixing the metal in said material as an insoluble silicate.
17. A process for the weighting of material comprising cellulose acetate, which consists in swelling and impregnating said material with a salt of a weighting metal in solution, and subsequently treating with a soluble phosphate and a soluble silicate to fix the metal in said material in the form of its corresponding insoluble salts.
18. A process for the weighting of material comprising cellulose acetate, which consists in swelling and impregnating said material with a chloride of a weighting metal in solution, and subsequently treating to fix the metal in said material as an insoluble salt.
19. A process for the weighting of material comprising cellulose acetate, which consists in swelling and impregnating said material with stannic chloride in solution, and subsequently treating to fix the tin in said material as an insoluble salt.
20. A process for the weighting of material comprising cellulose acetate, which consists in swelling and impregnating said material with stannic chloride in solution, and subsequently treating with alkali silicate to fix the tin in said material as an insoluble silicate.
21. A process for the weighting of material comprising cellulose acetate, which consists in swelling and impregnating said material with stannic chloride in solution, and subsequently treating with an alkali phosphate and an alkali silicate to fix the tin in said material in the form of its corresponding insoluble salts.
22. A process for the weighting of material comprising cellulose acetate, which consists in swelling and impregnating said material at a temperature of from 40-65° C. with stannic chloride in solution, and subsequently fixing the tin in said material as an insoluble salt.
23. A process for the weighting of material comprising cellulose acetate, which consists in swelling and impregnating said material at a temperature of from 40-65° C. with stannic chloride in solution, and subsequently fixing the tin in said material as an insoluble silicate.
24. A process for the weighting of material comprising cellulose acetate, which consists in swelling and impregnating said material at a temperature of from 40-65° C. with stannic chloride in solution, and subsequently treating with a soluble phosphate and a soluble silicate to fix the tin in said
- material in the form of its corresponding insoluble salts.
25. A process for the weighting of material comprising cellulose acetate, which consists in swelling and impregnating said material at a temperature of from 40-65° C. with stannic chloride in solution, and subsequently treating at a lower temperature to fix the tin in said material as an insoluble salt.
- In testimony whereof, we have hereunto subscribed our names.
- CAMILLE DREYFUS.  
H. PLATT.
- 75
- 80
- 85
- 90
- 95
- 100
- 105
- 110
- 115
- 120
- 125
- 130